

## 1

3,835,035

**METHOD OF PURIFYING LUBRICATING OILS**  
Morton Fainman, 11200 Homedale St., Los Angeles,  
Calif. 90049, and Charles Strouse McAuley, 9579  
Casanes Ave., Downey, Calif. 90240  
No Drawing Filed July 30, 1973, Ser. No. 383,706  
Int. Cl. C10m 11/00

U.S. CL. 208—181

30 Claims

### ABSTRACT OF THE DISCLOSURE

A method of purifying used lubricating oils comprising the following steps:

1. Admixing the used lubricating oil with a mutually soluble predominantly hydrocarbon liquid diluent which preferably has a boiling range within the temperature region of about 100° F. to about 550° F.;
2. Admixing the diluted lubricating oil with a water miscible alcohol and water mixture containing a small amount of an acid, and
3. Centrifuging to remove sludge and metal compounds from the oil and to separate the diluted oil phase from the alcohol-water phase to provide a purified organic layer having a low ash content.

The United States and other industrialized countries are faced with an increasing scarcity and increased cost of petroleum and petroleum products. Paradoxically, the industrial nations of the world are also faced with tremendous problems in utilizing used petroleum products without contaminating the environment.

Used high viscosity index lubricants, as employed for automobile lubrication, present a tremendous problem to the environment. Such lubricants commonly contain relatively large amounts of various detergents and extreme pressure additives in the form of polyvalent metal soaps as well as lead compounds, oxidized carbonaceous materials, water, etc. Due to their relatively high content of various additives, used lubricating oils cannot be burned simply without seriously polluting the air. Thus, literally millions of gallons of used lubricants are discarded annually because there is no economical way to recycle them.

Various methods have been employed to clean waste lubricating oils so that they may be reused. In general, these methods currently have been unsuccessful due primarily to economic factors.

Due to the change in the composition of lubricating oils through addition of additives such as soaps, E.P. agents, VI improvers and polymeric dispersants, the quantity of lubricating oil which can be recovered economically by reclaiming procedures has decreased. Thus, at present, the yield of lubricating oil which can be obtained by reclaiming is in the order of 50% or less of the recoverable organic material. Due to the severity of treatment, a substantial quantity of the recoverable organic material in the oil is lost. This makes the reclaiming procedure less economical and also results in the production of an increased quantity of sludge and by-products whose disposal causes contamination of the environment.

In one method of treatment which has been used, the used lubricating oil is first treated with caustic at an elevated temperature such as 400° F. to 600° F. to drive off water and to break soaps in the oil as well as to neutralize the oil. Also, in the course of heating, the light ends are flashed off and are generally burned. After the heating procedure, the oil is then cooled to about 100° F. or less and a small quantity of concentrated sulfuric acid is added. After settling, the bottoms are drawn off which contain an acid sludge comprising sul-

## 2

furic acid and dissolved sulfonates and oxygenated hydrocarbons. The sludge, which may constitute about 5 to 20% by weight of the used oil being treated, is disposed of by being placed in a closed container to prevent the escape of acid fumes. The sludge is then dumped. Due to the noxious properties of acid sludge, it is presently very difficult to find a land-fill which will accept material of this type. For example, in the Los Angeles area, acid sludge is hauled to San Diego where there is a landfill having a high lime content which will accept acid sludge.

After removal of the acid sludge from the oil, the top oil is then generally heated and finely divided clay is added at a temperature of about 350° F. The mixture of clay and top oil is then taken to a temperature of about 600° F. in a heater and after being held at this temperature for sufficient time is cooled to about 350° F. or less and passed through a filter press.

The above procedure, which is one of the procedures used for reclaiming lubricating oil, gives, at best, a yield of only about 50% reclaimed oil based on the weight of the used oil which was treated. The procedure produces large quantities of acid sludge which is difficult to dispose of. Also, the process requires substantial heating, which is expensive, as well as the use of expensive chemicals which are not recoverable.

Another procedure which has been used for treatment of used lubricating oils involves treatment of the oil with lime and finely divided clay. A still further procedure involves treatment of the oil with a mixture of caustic and sodium silicate. All of the above noted procedures give a yield of purified oil of 50% or less based on the weight of the used oil being treated together with the production of 5% to 20% of light ends or tops which are burned. Additionally, all of the above procedures produce substantial quantities of sludge which cannot be recycled and must be dumped.

In providing a solution to the aforementioned problems, the present process for the purification of used lubricating oils is economical—providing a yield of about 80 to about 95% or more of the recoverable organic material in the used oil—and also produces a very small amount of residue composed of polyvalent metal compounds in admixture with oxidized hydrocarbons and all of the myriad materials which are found in the sludge from used lubricating oils. Thus, the process provides a means for substantially reducing environmental pollution resulting from the dumping of waste oil. Also, the process provides a new source of high viscosity index oils which are presently in short supply and are urgently needed in industrialized countries for automotive lubrication.

In accord with the process, used lubricating oils, which may be collected from various sources, such as independent service stations throughout a large area, are first admixed with a predominantly hydrocarbon liquid diluent which preferably has a boiling range within the temperature region of about 100° F. to about 550° F. The liquid diluent may be either aromatic or aliphatic and is mutually soluble with the used hydrocarbon lubricating oil undergoing treatment. The function of the liquid diluent in the process, as envisioned, is to lower the viscosity of the used lubricating oil and to change the characteristics of the used lubricating oil dispersion to thereby facilitate the contact, with the used lubricating oil in the subsequent steps of the process, of a water miscible alcohol-water mixture.

The term "predominantly," as used in defining the hydrocarbon content of the liquid diluent, refers to a liquid whose hydrocarbon content is about 90% by weight or greater. Impurities which may be present in the liquid diluent, which may be recycled light ends from the purified lubricating oil, may include, for example, small

quantities of sulfur-containing compounds, such as mercaptans, and oxygenated hydrocarbons such as aldehydes or ketones. The impurities which may be present in the liquid diluent will vary depending on the makeup of the used lubricating oil which is the source of the recycled light ends. Thus, the above listing of impurities is not intended to be all inclusive.

Preferably, the predominantly hydrocarbon liquid diluent has a boiling range within the temperature region of about 100° F. to about 500° F. although lower boiling hydrocarbon liquids, such as liquid propane, may also be employed. The purified lubricating oil produced in accord with the process may be subjected to distillation. In the course of the distillation, the light or naphtha ends may be recycled to the process to serve as the predominantly hydrocarbon liquid diluent for the used lubricating oils being treated. Thus, after initial start-up, the process will be self-sustaining with sufficient naphtha light ends being supplied through distillation of the purified oil or organic phase to satisfy the need for liquid diluent in diluting the as received used lubricating oil.

The quantity of the liquid diluent which is employed in diluting the as received used lubricating oil may be varied in accord with the process. A particularly practical range of liquid diluent with respect to used oil ranges from about 1:1 to about 1:2 by volume, although other dilutions may be used, if desired, such as 2:1 or even 4:1 depending, for example, on the solids content and viscosity of the used drain oil undergoing treatment and the efficacy of the diluent liquid in furthering contact by the extraction solvent.

Generally, it is desirable to use the smallest amount of diluent possible since an increase in the amount of diluent makes the subsequent separation of the diluent and the oil more involved and costly. For example, when the amount of diluent is increased, the size of the separation equipment, such as distillation columns, etc., must also be proportionately increased which causes an increase in the cost of the processing equipment.

After dilution of the used lubricating oil undergoing treatment with a predominantly hydrocarbon liquid diluent, as described, the diluted lubricating oil is then contacted with a mixture of water, a water miscible alcohol, and a small quantity of an acid. Although not bound by any theory, it is believed that the acid functions to displace polyvalent metal ions from the various metallic soaps which are present in the diluted lubricating oil undergoing treatment. As the polyvalent metal ions are displaced from the soaps by hydrogen ions, the soaps are converted to lower molecular weight acids. With the decrease in molecular weight, the solubility of the resulting acids in the diluted lubricating oil is decreased while their solubility in the water-alcohol phase is increased. This phenomena is believed to facilitate the extraction of the metal soaps from the diluted lubricating oil through contact with the water miscible alcohol-water mixture. Also, for reasons which are not understood, the resultant change in the dispersant composition of the oil phase releases the peptized solids which may then be removed by centrifugation as will be described.

Among the water miscible alcohols which may be used in this step of the process are methanol, ethanol, isopropyl alcohol, *n*-propyl alcohol, *sec*-butyl alcohol, and *tert*-butyl alcohol. The higher alcohols, such as amyl alcohol and also alcohols having a lower water solubility such as *n*-butyl alcohol, have such a low solubility in water that they are generally ineffective in the present process. Thus, the water miscible alcohols which are suitable in the process, including polyhydric alcohols, generally have a solubility of about 20% or more by volume in water.

Of the various alcohols, it was found that isopropyl, ethyl, *n*-propyl and *tert*-butyl alcohol functioned best in the performance of the process. Moreover, it was found that alcohol-water mixtures containing from about 40 to about 60% by volume of alcohol were generally more

effective than mixtures containing either more or less alcohol in relation to the amount of water in the alcohol-water mixture.

In describing the present process, it should be emphasized that the material undergoing treatment, i.e., used lubricating oil, is not a homogeneous material. Thus, in practice, the specific operating conditions employed may be varied to suit the particular batch of lubricating oil which is being treated. For example, if the batch of lubricating oil undergoing treatment has a relatively high water content, this factor may be taken into consideration in determining the ratio of alcohol to water in treating the lubricating oil after it has been diluted with a predominantly hydrocarbon liquid diluent as described.

In determining the optimum process conditions for a particular batch of used lubricating oils, the lubricating oils may, for example, be collected in a relatively large holding tank. When the holding tank is full, representative samples may then be taken and analyzed with a view to determining the optimum process conditions for treating the used oil in that tank. By way of example, the behavior of the samples may be determined in considering how much of the predominantly hydrocarbon liquid diluent available for processing to mix with the used lubricating oil on a volume-to-volume relationship to obtain the optimum basis for handling and centrifugation. Also, to determine optimum conditions, samples of the used lubricating oil in the holding tank may be treated on a small scale according to the present process to determine the conditions which provide the greatest reduction in the ash content of the oil being treated and the greatest yield of purified oil.

A particularly suitable quantity of the water miscible alcohol-water mixture is about one volume of the mixture for each volume of the diluted used lubricating oil for one-stage extraction of the diluted lubricating oil. The diluted lubricating oil may be subjected to multiple-stage extraction with a water miscible alcohol-water mixture, as described, and also the quantity of the alcohol-water mixture may be varied, for example, from about one-half volume of alcohol-water mixture to two volumes of the diluted lubricating oil to higher volume ratios in excess of 1:1. In general, the volume of the water miscible alcohol-water mixture is kept as low as possible since this simplifies the subsequent processing steps in terms of equipment size, cost, etc.

Various water soluble acids (preferably inorganic acids) may be employed in the alcohol-water mixture used in treating the diluted lubricating oil. To illustrate, hydrochloric acid, sulfuric acid, nitric acid and phosphoric acid have all been employed and found suitable. Although not bound by any theory, it is believed that the decomposition of the polyvalent metal soaps (generally bivalent metal soaps) and the removal of the organic acids from the organic layer to the alcohol-water layer reduces the efficacy of the non-ionic dispersants remaining in the oil to maintain the micellar configuration necessary to keep the solids and sludge in dispersed form in the diluted oil.

In displacing polyvalent metal ions with hydrogen ions to convert soaps in the treated oil to lower molecular weight acids, the displaced metal ions may form salts with the anionic portion of the treating acid. To promote the migration of such salts into the alcohol-water phase, the treating acid is preferably one which does not contain a bulky anionic group, e.g., a sulfonic acid group, which would enhance the solubility in the oil phase of salts formed with the displaced polyvalent metal ions and, thereby, inhibit migration of such salts into the alcohol-water phase.

In general, the quantity of the acid which is used is sufficient to displace the polyvalent metal ions from the soaps within the oil. As an example, in treating a diluted used lubricating oil (containing one-half volume of used lubricating oil admixed with one-half volume of a liquid predominantly hydrocarbon diluent) by mixing with one

volume of a 50:50 volume ratio water miscible alcohol-water mixture, it was found that the use of three milliliters of an acid, e.g., concentrated hydrochloric acid, for each 100 mls. of the alcohol-water mixture gave satisfactory results.

Agitation is generally employed during the treatment of the diluted lubricating oil with the alcohol-water mixture containing an acid. For example, the agitation may be provided by mixing within a large vessel through use of a mixing impeller, in a continuous, metered in-line mixing device such as a gear pump or homogenizer, or by using any other mixing procedure.

The agitation of the diluted lubricating oil and alcohol-water mixture is generally carried out until an emulsion forms which indicates that the diluted oil has been thoroughly contacted with the alcohol-water mixture. The emulsion is generally unstable and is broken during the subsequent centrifuging step. If the emulsion is not broken during centrifuging, this is undesirable since the process yield is reduced by trapping of recoverable oil in the emulsion phase. It is preferred that the formation of a stable emulsion which is not broken by centrifuging be kept to a minimum. This may be accomplished by taking representative samples of the used oil being treated and then varying the process parameters on a small scale to determine the optimum yield conditions. By determining the optimum processing conditions for a particular used oil, the formulation of a stable emulsion may be minimized to provide the maximum yield of recoverable organic material in the oil.

Following the treatment of the diluted lubricating oil with the alcohol-water mixture, as described, the resulting mixture is then fed to a centrifuge for separation of the sludge from the lubricating oil and also separation of the alcohol-water mixture from the organic mixture of liquid diluent and lubricating oil. Industrial centrifuges are well known and any of the various types of centrifuges may be used in the present process. The resultant mixture is simply fed into the centrifuge with the sludge depositing out on the walls of the centrifuge while the alcohol-water mixture is taken off through one outlet and the organic mixture of liquid diluent and lubricating oil is removed through another outlet. Periodically, the sludge formed on the interior of the centrifuge may be removed by ejection, backwashing or by spraying the interior of the centrifuge bowl with a jet of water. These various procedures for removing solids from industrial centrifuges are well known.

The alcohol-water stream which is taken from the centrifuge contains organic acids. Depending upon the acid content of the alcohol-water mixture, the mixture of water miscible alcohol and water may be recycled directly to the process for use in treatment of used lubricating oil diluted with a predominantly hydrocarbon liquid, as described. However, the alcohol-water stream may also first be subjected to a clean-up operation before return to the process. Any conventional procedure may be used for cleaning the alcohol-water stream to remove organic acids such as extraction of the organic acids, ion exchange, distillation or neutralization followed by distillation of the alcohol followed by addition of fresh make up water to the alcohol, etc.

The mixture of purified lubricating oil and predominantly hydrocarbon liquid diluent may be used as a low ash fuel or the mixture may be separated through conventional distillation. The naphtha fraction from the distillation may, as described previously, be recycled for use in the process in diluting the used lubricating oil. The purified lubricating oil fraction from the distillation may be used as the base stock in compounding new lubricating oils.

A convenient and accurate way of measuring the effectiveness of the present process in terms of the purity of the lubricating oil obtained is to compare the ash content of the as-is used lubricating oil with the ash

content of the purified lubricating oil product obtained from the process. Based on experiments carried out with two used lubricating oils obtained from different sources, the present process may provide a reduction in the ash content of the oil of 80 to 90%. For example, an ash content of about 2% in the as received used oil was reduced to about 0.2% in the purified oil. In addition, of course, there is a reduction in the additive content of the oil which simplifies further processing of the purified oil using conventional refinery procedures.

10 The residue from the process, which consists of the various materials that are present in the sludge of a used lubricating oil may constitute about 3% by weight of the as received used lubricating oil. Thus, the residue is 15 only a very small fraction of the weight of the used lubricating oil. By greatly reducing the weight of the residue removed from the used lubricating oil during purification, the process does not present the problems of waste disposal which have plagued previous attempts to 20 process used lubricating oils.

25 The residue from the process has a high metallic content, predominantly lead, and, thus, represents a potentially valuable source of metals. In view of the large quantity of used lubricating oil which is generated by 30 crankcase drainings from automobiles, the process residue from all the used oil would be quite sizable in terms of total weight of metals, even though the residue represents only a small percentage by weight of the used lubricating oil being treated. Thus, the residue may be 35 processed, where economically feasible, to recover its metal fractions.

If desired, the present process may be used in conjunction with the process of our prior copending U.S. Patent Application, Ser. No. 336,733, filed June 4, 1973, the 35 subject matter of which is incorporated herein by reference. As disclosed in our copending application, a used lubricating oil is purified by mixing the used lubricating oil with a mutually soluble predominantly hydrocarbon liquid diluent which preferably has a boiling range within 40 the temperature region of about 100° F. to about 550° F.; then admixing the diluted lubricating oil with a water miscible alcohol and water mixture containing a small amount of an ammonium or alkali metal base, and centrifuging to remove sludge and metal compounds from 45 the oil and to separate the diluted oil phase from the alcohol-water phase to provide a purified organic layer having a low ash content.

From a comparison of the present process with that of prior Application 336,733, it can be observed that the general conditions of the two processes are the same. However, in our prior process, the alcohol-water mixture contains a small amount of an ammonium or alkali metal base while in the present process the alcohol-water mixture contains a small amount of an acid. As disclosed in our 50 prior application, various water soluble ammonium and alkali metal bases may be employed in the alcohol-water mixture used in treating the diluted lubricating oil. To illustrate, ammonium carbonate, sodium carbonate, potassium carbonate, lithium carbonate, and sodium hydroxide have all been employed and found suitable. Of the various bases which have been employed, sodium carbonate and sodium phosphate are preferred. Although not bound by any theory, it is believed that the carbonate and phosphate anions are particularly effective in reducing the solubility of the polyvalent metal cations 55 which are displaced from the metallic soaps in the diluted lubricating oil by the monovalent ammonium and alkali metal ions, and in reducing the efficacy of the non-ionic dispersants remaining in the oil to maintain the micellar configuration necessary to keep the solids and sludge in dispersed form in the diluted oil. Surprisingly, closely related anions, such as the bicarbonate ion, were found to be less effective in the process than the carbonate ion.

In the practice of the process of our prior application, 60 it has been found that the use of excessive quantities of the

water soluble ammonium or alkali metal base actually cause a reduction in the overall efficiency of the process, i.e., by producing a purified oil whose ash content is higher than that which is obtained through use of a smaller quantity of the base. It is believed that this result occurs because of the presence of non-ionic detergents which are also present in used lubricating oils. When excessive quantities of the monovalent cation, e.g., sodium base are employed, which are in excess of that required to displace the polyvalent metal cations from soaps within the oil, the additional sodium is believed to be taken up by the non-ionic detergents. This would increase the ability of the non-ionic detergents to suspend sludge and metal within the oil. As a result, the purified oil obtained from the process will have a higher ash content than that obtained by using a lesser quantity of the ammonium or alkali metal base. Thus, it is preferred that the quantity of the ammonium or alkali metal base is sufficient to displace the polyvalent metal ions from the soaps within the oil but that the base not be present in any great excess of that amount.

After treatment of a used lubricating oil according to the process of our prior Application 336,733, the ash content of the oil is reduced by as much as about 80 to 90%. However, the content of monovalent cations, e.g., sodium, in the thus purified oil is generally high due to the presence of the base in the alcohol-water mixture used in the process. When a purified oil or oil phase resulting from treatment according to our prior process is then subjected to a second stage treatment using the conditions of the present process, there is a further marked reduction in the ash content by as much as another 80 to 90%. Thus, if the as received oil had an ash content of about 2%, the first stage treatment according to our prior process may reduce the ash content to about 0.2%. When the thus purified oil is then subjected to a second stage treatment according to the present process, its ash content may be further reduced to about 0.02%.

Surprisingly, it has been found that such a second stage treatment according to the present process is much more effective than a second stage treatment using the same general conditions used in the first stage treatment. Thus, for example, when oil treated according to our prior process (Ser. No. 336,733) is treated in a second stage, using these same general conditions, the percentage reduction in ash content achieved by the second stage is not nearly as high as that achieved by the first stage treatment. However, when the conditions of the present process are used for the second stage treatment, the percentage reduction in ash content in the second stage is of the same general magnitude as the percentage reduction in ash content in the first stage. Thus, there is a unique coaction between the present process and the process of our Application 336,733 when the two processes are used as separate treatment stages in a multi-stage oil treatment process.

The examples described in the following tables were generally conducted by mixing a measured volume of a used drain oil with a measured volume of an indicated predominantly hydrocarbon liquid diluent. After mixing the drain oil and diluent, the diluted oil was then admixed with a specified alcohol-water mixture, thoroughly agitated, and then centrifuged for four hours.

The method of centrifuging used was a modification of ASTM method D1796-62. In centrifuging, 100 ml. cone shaped tubes (described in the ASTM method) were first filled with the resultant mixture formed from the diluted drain oil and the mixture of alcohol with water. The cone shaped tubes and their contents were then whirled in a Precision Oil Centrifuge (Catalog No. 67343) to produce a relative centrifugal force of 800 at the tips of the tubes.

On completion of the centrifuging, the contents of the tubes had separated into several layers. At the bottom of the tube was a layer of sludge which had been removed from the drain oil by the process of the invention. Above

the lower sludge layer was a water miscible alcohol-water layer and above this layer was an organic layer containing a purified organic phase of the predominantly hydrocarbon liquid diluent with the purified drain oil. This upper layer is termed the organic layer. In some of the examples, an emulsion or dispersion formed which was not completely broken by the centrifuging and which appeared within the organic or the alcohol-water phase or as a layer at the interface between the organic layer and the alcohol-water layer.

The yield of recoverable organic material in volume percent of the drain oil was determined by measuring the volume of the purified organic layer and subtracting the volume of the hydrocarbon liquid diluent from this volume. The remaining volume, which is the volume of the recovered organic material from the drain oil, was then divided by the original volume of the drain oil to determine the percent yield of recoverable organic material. In some instances, as indicated in the tables, the yield of recoverable organic material from the drain oil was observed to be in excess of 100%. In these instances, a dispersion or emulsion was observed and there had obviously been a transfer of material into the organic layer which produced the high reading.

After centrifuging, as described above, a sample was removed from the organic phase using a 100 ml. syringe fitted with an 8-inch needle. The sample from the organic phase was then analyzed to determine its solids content and the ash content of the solids. The ash content of the purified drain oil was then converted to an ash content based on the weight of the original drain oil by multiplying the ash content of the solids by the percent solids in the original oil. This, then, permitted a direct evaluation of the process in terms of the percentage reduction which was obtained in the ash content.

In determining the percentage of solids in the drain oil or the purified organic layer a ten gram sample was weighed into a soft, crimped aluminum dish having a diameter of 2 1/8 inches, a depth of 5/8 inches and a finger-grip handle. The dish was placed on a Corning Pyroceram 600-watt hotplate with a temperature dial set to produce a surface temperature of approximately 450° F. and preheated to the operating temperature. Heating at about 450° F. was maintained for one hour, after which the dish was removed, cooled to ambient temperature, and reweighed. The percent of solids was then determined by dividing the final weight of the residue by the weight of the sample and multiplying by 100.

The ash content of the drain oil or the purified organic layer was determined by ASTM method D482-63. In determining ash, the analytical problems which are associated with the presence of phosphorus and lead compounds were disregarded since the results were used on a comparative basis. In other words, any error produced by the presence of phosphorus or lead would have a similar effect in the ash analysis of the used drain oil as in the ash determination for the purified organic liquid. Thus, the errors, if any, would not affect the validity of the comparison of the ash content of the used drain oil with that of the purified organic liquid.

The method for determining ash consists of weighing a sample of the material to be ashed into a 30 ml. porcelain crucible. The material in the crucible is then ignited and allowed to burn until only ash and carbon remain. The carbonaceous residue is then reduced to an ash by heating in a muffle furnace at 775° C., followed by cooling and weighing. As determined by this method, the ash content primarily indicates the metals content of the sample expressed in terms of the inorganic salts of the metals which are predominantly phosphates, oxides, silicates, sulfates, etc.

In determining the ash content of the purified drain oil corrected to the weight of the used drain oil, the solids content and the ash content of the used drain oil were

determined as a percentage of the weight of the drain oil sample. The ash content of the purified organic layer was also determined as a percentage based on the solids content of the sample from the purified organic layer. Conveniently, the weight of solids of the purified organic layer was determined and these solids were then burned to determine the ash content of the solids. The ash content of the purified organic layer, expressed as a percent of the solids in the sample, is then converted to weight percent ash based on the drain oil by multiplying by the percent of solids in the used oil.

The basis for the conversion of the ash in the purified organic layer to percent ash based on the used drain oil is based on the fact that the ash is contained in the solids and the total solids content of both the drain oil and the purified organic layer is relatively constant and is only slightly affected by the present process. In the course of heating at about 450° F. to determine solids, the liquid hydrocarbon diluent in the sample from the purified organic layer is driven off. Thus, the solids which remain are those obtained from the used drain oil being treated. Likewise, in determining solids in the used drain oil, the heating at about 450° F. drives off the light fractions as well as any water present in the drain oil. The solids which remain are largely hydrocarbons which have a boiling point in excess of 450° F., and these solids are almost entirely recovered by the present process.

The solids content changes slightly as a result of the present process since the sludge and metals which are removed from the used drain oil are solids. However, the weight of the solids which are removed is very small in comparison to the total weight of solids composed mainly of hydrocarbons whose boiling point is in excess of 450° F. For these reasons, the assumption that the solids content from the drain oil remains fixed throughout the process is reasonably valid and any errors resulting from this approximation are within an error of about 5% of the observed values, i.e.,  $\pm 0.05$  times the observed values.

TABLE I  
Drain oil of 1.44% (wt.) ash

| Example number.                           | 1    | 2    | 3    |
|-------------------------------------------|------|------|------|
| Drain oil (mls.)                          | 25   | 25   | 50   |
| Naphtha diluent (mls.)                    | 25   | 25   | 50   |
| 50% (vol.) isopropyl alcohol-water (mls.) | 50   | 50   | —    |
| Concentrated HCl (ml./100 ml. alc-water)  | 3    | —    | —    |
| Recovery of drain oil (vol. percent)      | 102  | 98   | 98   |
| Ash of recovered drain oil (wt. percent)  | 0.84 | 0.36 | 0.92 |
| Dispersion (organic layer)                | None | None | Yes  |
| Dispersion (alcohol layer)                | Yes  | None | —    |

As shown in Table I, Examples 1-3 are each concerned with a drain oil having an ash content of 1.44% by weight. In Example 1, the ash content was reduced to 0.84%, based on the weight of original drain oil, while in Example 2 the ash content was reduced to 0.36%. The striking effect of adding an acid to the alcohol-water mixture is illustrated by the results of Example 2 in which all of the process conditions were otherwise the same as in Example 1. Example 1. Example 3 illustrates the effect of dilution in which 50 mls. of drain oil were admixed with 50 mls. of naphtha diluent and then centrifuged directly without being contacted by the alcohol-water mixture. As shown, there was some reduction in the ash contained by dilution of the drain oil with a hydrocarbon diluent and centrifuging. However, this reduction in ash was far less than that obtained, for example, in Example 2 where the diluted drain oil was thoroughly admixed with 50 mls. of a 50% by volume

mixture of isopropyl alcohol and water which contained a small quantity of an acid.

TABLE II

Drain oil—1.73% (wt.) ash (dilution effect)

| Example number.                          | 4    | 5    | 6    | 7    | 8    |
|------------------------------------------|------|------|------|------|------|
| Drain oil (mls.)                         | 100  | 66.7 | 50   | 33.3 | 20   |
| Naphtha diluent (mls.)                   | 0    | 33.3 | 50   | 66.7 | 80   |
| Recovery of drain oil (vol. percent)     | 99.8 | 99.1 | 99.5 | 99.4 | 99.5 |
| Ash of recovered drain oil (wt. percent) | 1.60 | 1.30 | 1.22 | 1.11 | 0.90 |
| Dispersion (organic layer)               | Yes  | Yes  | Yes  | Yes  | Yes  |

Table II illustrates the effect of dilution, i.e., variations in the amount of hydrocarbon diluent with respect to the amount of drain oil, without a following treatment with an alcohol-water mixture. As shown in Example 4, some reduction in ash content was obtained merely by centrifuging the drain oil. As the quantity of hydrocarbon diluent was increased in Examples 5-8 while the quantity of drain oil was decreased, there was a continuing reduction in the ash content of the recovered drain oil. However, there was still a substantial amount of ash in the treated oil which indicates that dilution, while important, is not sufficient to purify the drain oil without the added step of contacting the diluted drain oil with the alcohol-water mixture which contains an acid.

TABLE III

Drain oil—1.73% (wt.) ash (variation in alcohol concentration)

| Example number.                          | 9    | 10   | 11   | 12   |
|------------------------------------------|------|------|------|------|
| Drain oil (mls.)                         | 25   | 25   | 25   | 25   |
| Naphtha diluent (mls.)                   | 25   | 25   | 25   | 25   |
| Vcl. percent isopropanol in water        | 30   | 40   | 50   | 60   |
| Isopropanol-water (mls.)                 | 50   | 50   | 50   | 50   |
| Concentrated HCl (ml./100 ml. alc-water) | 4    | 4    | 4    | 4    |
| Recovery of drain oil (vol. percent)     | 98   | 96   | 98   | 98   |
| Ash of recovered drain oil (wt. percent) | 0.53 | 0.46 | 0.41 | 0.41 |
| Dispersion (organic layer)               | None | None | None | None |
| Dispersion (alcohol layer)               | None | Some | Some | None |

Examples 9-12, shown in Table III, illustrate the effect of variations in the alcohol concentration of the alcohol-water mixture which was employed. For the particular drain oil undergoing treatment, which contained 1.73% by weight of ash, it was observed that an isopropyl alcohol concentration of about 40 to about 60% by volume in the alcohol-water mixture was most effective. Using these concentrations, there was a very marked reduction in the ash content of the treated oil and a very clean separation between the organic layer and alcohol layer. At lower concentrations of isopropanol, the process was less effective as evidenced by a higher ash content in the recovered oil.

TABLE IV

Drain oil—1.73% (wt.) ash (variations in alcohol)

| Example number.                          | 13      | 14         | 15           |
|------------------------------------------|---------|------------|--------------|
| Drain oil (mls.)                         | 25      | 25         | 25           |
| Naphtha Diluent (mls.)                   | 25      | 25         | 25           |
| Alcohol                                  | Ethanol | n-Propanol | Tert-Butanol |
| Vol. percent alcohol in water            | 60      | 50         | 50           |
| Alcohol-water (mls.)                     | 50      | 50         | 50           |
| Concentrated HCl (ml./100 ml. alc-water) | 3       | 3          | 3            |
| Recovery of drain oil (vol. percent)     | 96      | 94         | 108          |
| Ash of recovered drain oil (wt. percent) | 0.50    | 0.37       | 0.35         |
| Dispersion (organic layer)               | None    | None       | None         |
| Dispersion (alcohol layer)               | None    | None       | None         |

Table IV sets forth the results obtained in Examples 13-15 in which the alcohol present in the alcohol-water mixture was varied. As illustrated, all of the various alcohols tested were found to be effective and, in addition to *iso*-propanol, ethanol, *n*-propanol and *tert*-butanol were found to be particularly effective.

TABLE V  
Drain oil—1.73% (wt.) ash (variation in acid)

| Example number                         | 16        | 17                                   | 18                     | 19                                   | 20               | 21                   |
|----------------------------------------|-----------|--------------------------------------|------------------------|--------------------------------------|------------------|----------------------|
| Drain oil (mls.)                       | 25        | 25                                   | 25                     | 25                                   | 25               | 25                   |
| Naphtha diluent (mls.)                 | 25        | 25                                   | 25                     | 25                                   | 25               | 25                   |
| 50% vol. isopropanol-water (mls.)      | 50        | 50                                   | 50                     | 50                                   | 50               | 50                   |
| Acid (ml./100 ml. alc-water)           | 3 ml. HCl | 2 ml. H <sub>2</sub> SO <sub>4</sub> | 3 ml. HNO <sub>3</sub> | 3 ml. H <sub>3</sub> PO <sub>4</sub> | 2 ml. 88% formic | 3 ml. glacial acetic |
| Recovery of drain oil—vol. percent     | 96        | 98                                   | 96                     | 98                                   | 98               | 98                   |
| Ash of recovered drain oil—wt. percent | 0.36      | 0.41                                 | 0.45                   | 0.62                                 | 0.75             | 0.85                 |
| Dispersion (organic layer)             | None      | None (gel)                           | None                   | None                                 | None             | None                 |
| Dispersion (alcohol layer)             | None      | None                                 | Yes                    | None                                 | Slight           | Slight               |

Table V describes the results obtained in Examples 16–21 in which various acids were employed in the alcohol-water mixture. As shown, all of the acids which were tested were found to be effective and hydrochloric acid and nitric acid were particularly effective. The optimum alcohol to water ratios were not determined for each acid as in the case of hydrochloric acid as set forth in Table III. The separation between the organic layer and alcohol layer was clean in Examples 16 and 19 with some gel formation in the organic layer in Example 17 and the formation of some dispersion in the alcohol layer in Examples 18, 20 and 21.

TABLE VI

Drain oil—1.73% (wt.) ash (variation in diluent)

| Example number                           | 22    | 23     | 24         |
|------------------------------------------|-------|--------|------------|
| Drain oil (mls.)                         | 25    | 25     | 25         |
| Hydrocarbon diluent                      | Kero- | Xylene | Dehydrated |
| Diluent (mls.)                           | 25    | 25     | 25         |
| 50% vol. isopropyl alcohol-water (mls.)  | 50    | 50     | 50         |
| Concentrated HCl (ml./100 ml. alc-water) | 3     | 3      | 3          |
| Recovery of drain oil (vol. percent)     | 94    | 98     | 98         |
| Ash of recovered drain oil (wt. percent) | 0.36  | 0.36   | 0.36       |
| Dispersion (organic layer)               | None  | None   | None       |
| Dispersion (alcohol layer)               | None  | None   | None       |

Table VI illustrates the results obtained from Examples 22–24 in which the hydrocarbon diluent was varied. These examples demonstrate that a wide variety of hydrocarbon diluents may be employed in the process in obtaining a marked reduction in the ash content of the treated oil. The use of kerosene as a diluent demonstrates that relatively high molecular weight solvents are suitable while the use of xylene demonstrates that an aromatic diluent may likewise be employed.

TABLE VII

Drain oil—1.73% (wt.) ash (variation in acid concentration)

| Example number                           | 25   | 26   | 27   | 28   | 29   |
|------------------------------------------|------|------|------|------|------|
| Drain oil (mls.)                         | 25   | 25   | 25   | 25   | 25   |
| Naphtha diluent (mls.)                   | 25   | 25   | 25   | 25   | 25   |
| 50% isopropanol-water (mls.)             | 50   | 50   | 50   | 50   | 50   |
| Concentrated HCl (ml./100 ml. alc-water) | 0.5  | 1.0  | 1.5  | 3.0  | 4.0  |
| Recovery of drain oil (vol. percent)     | 102  | 100  | 100  | 96   | 98   |
| Ash of recovered drain oil (wt. percent) | 0.60 | 0.49 | 0.52 | 0.36 | 0.41 |
| Dispersion (organic layer)               | None | None | None | None | None |
| Dispersion (alcohol layer)               | Yes  | Some | None | None | None |

Examples 25–29, shown in Table VII, illustrate the effect on the process of variations in the amount of the concentrated hydrochloric acid present in a 50% alcohol-water mixture. For the particular drain oil undergoing treatment, which contained 1.73% by weight of ash, it was observed that an acid concentration of 3 ml. of concentrated hydrochloric acid was most effective. This concentration gave the most marked reduction in the ash content of the treated oil and a very clean separation between the organic layer and alcohol-water layer.

15 TABLE VIII  
(Two-stage process)

| Example number                           | 30 (1st stage)                  | 31 (2nd stage) | 32 (2nd stage) |
|------------------------------------------|---------------------------------|----------------|----------------|
| Drain oil (mls.)                         | 25                              | 50             | 50             |
| Naphtha diluent (mls.)                   | 25                              | 50             | 0              |
| Vol. percent isopropanol in water        | 50                              | 50             | 50             |
| Isopropanol-water (mls.)                 | 50                              | 50             | 50             |
| Base (1.0 gm./100 ml. alc-water)         | Na <sub>2</sub> CO <sub>3</sub> | 3              | 3              |
| Concentrated HCl (ml./100 ml. alc-water) | 92                              | 98             | 98             |
| Recovery of drain oil (vol. percent)     | 0.30                            | 0.049          | 0.17           |
| Ash of recovered drain oil (wt. percent) | None                            | None           | None           |
| Dispersion (organic layer)               | None                            | Some           | Some           |

30 Table VIII illustrates the results of a two-stage purification procedure in which the first stage (Example 30) is carried out according to the process of our previous U.S. Application 336,733. In Example 30, 25 mls. of a used drain oil having an ash content of 1.73 weight percent was admixed with 25 mls. of a naphtha diluent and the mixture was then contacted with 50 mls. of a 50 percent by volume isopropanol-water mixture in the presence of a base containing a monovalent cation. Sodium carbonate was the base employed (although other bases may be used) at a concentration of one gram for each 100 ml. of the alcohol-water mixture. After agitation to insure intimate contact of the organic and alcohol-water phases, the overall mixture was centrifuged in the manner described previously to provide an organic layer consisting of the recovered drain oil and hydrocarbon diluent. The ash content of the recovered drain oil was 0.30% based on the weight of original drain oil and 92% by volume of the treated drain oil was recovered.

40 The organic layer provided by the procedure of Example 30 (a 50:50 volume mixture of recovered drain oil and naphtha diluent) was then employed as the starting material for a second stage treatment. In Example 31, the second stage treatment was the process of the present invention in which 50 mls. of the purified organic layer from the first stage was used as the starting material. As illustrated by Example 31, the use of the present process as the second stage to a first stage treatment according to the process of our application 336,733 reduced 45 the ash content of the purified oil from 0.30% to 0.49% by weight based on the weight of the original used oil. This is a drastic reduction which is much greater than the reduction obtained when both the first and second stages are conducted according to the process of application 336,733 or when both stages are conducted using the 50 conditions of the present process.

55 In Example 32, the alcohol was eliminated in a second stage treatment which are otherwise carried out using the conditions of the present process. As indicated, the elimination of the water miscible alcohol in Example 32 greatly reduced the effectiveness of the second stage treatment. While some further reduction of the ash content of the oil was achieved, the reduction was not nearly 60 as great as that obtained in Example 31.

TABLE IX  
Characteristics of hydrocarbon diluents

| Properties                                | Kero-sene | Naph-tha | Dehy-drated overhead | Xylene |
|-------------------------------------------|-----------|----------|----------------------|--------|
| Gravity, ° API                            | 41.5      | 47.3     | 45.0                 | 31.3   |
| Reid vapor pressure                       |           | 0.3      | 1.5                  |        |
| Sulfur, percent by wt.                    | <0.01     | <0.01    | 0.1                  | <0.01  |
| Flash point, tag closed cup (° F.)        | 152       | 104      | 60                   | 88     |
| Distillation, initial boiling pt., (° F.) | 380       | 311      | 180                  | 283    |
| End point (° F.)                          | 499       | 386      | 480                  | 293    |

5 10

Table IX illustrates the characteristics of the hydrocarbon diluents referred to in the various Examples. As indicated by Table IX and the Examples, a variety of diluents may be employed in the present process, ranging from aliphatics to aromatic and including a dehydrated overhead from a used drain oil.

To ascertain the nature of the metals found in used lubricating oils, and the effectiveness of the present process in reducing the content to these metals, the metals analysis set forth in Table X was conducted on the used drain oil which was treated in Example 30 having an ash content of 1.73 percent by weight. After a first stage treatment using the conditions of Example 30, i.e., the process of our prior application 336,733, the metals content of the purified oil was determined. Then, organic material obtained according to Example 30 (50-50 volume mixture of purified drain oil and naphtha diluent) was subjected to a second-stage treatment using the conditions of Example 31 (the present process) and the metals content of the purified oil from the second-stage treatment was determined. The metals content of the purified oil after both the first and second stage treatments is corrected to the weight of the original used oil (as is condition) in the same manner as described previously.

TABLE X  
Metals content of drain oil in parts per million

| Element                                                        | Original drain oil, 1.73% (wt.) ash | Treated oil                 |                             |
|----------------------------------------------------------------|-------------------------------------|-----------------------------|-----------------------------|
|                                                                |                                     | Example 30, 0.30% (wt.) ash | Example 31, 0.49% (wt.) ash |
| Lead                                                           | 5,000                               | 180                         | 43                          |
| Zinc                                                           | 1,500                               | 210                         | 24                          |
| Phosphorus                                                     | 860                                 | 260                         | 210                         |
| Calcium                                                        | 1,500                               | 110                         | 3                           |
| Iron                                                           | 390                                 | 120                         | 7                           |
| Magnesium                                                      | 420                                 | 50                          | 1                           |
| Barium                                                         | 440                                 | 130                         | 30                          |
| Potassium                                                      | 230                                 | 10                          | Nil                         |
| Sodium                                                         | 20                                  | 250                         | Nil                         |
| Others (Cr, Sb, Cd, Sn, B, Mn, Cu, Ni, Al, Bi, Mo, Li, Ag, Ti) | 210                                 | 50                          | 45                          |
| Total                                                          | 10,570                              | 1,379                       | 363                         |

40 45 50 55 60 65 70 75

The above data demonstrate that the present process (as exemplified by Example 31) was effective in reducing the content of all the various metals found in drain oil. Further, the data demonstrate that the present process is very effective as a second-stage treatment to a purified oil after a first-stage treatment according to the process of our prior application 336,733 as exemplified by Example 30. As would be expected, there was an increase in the sodium content of the oil after the first-stage treatment since the base present in the alcohol-water mixture contained sodium. However, after the second-stage treatment, the sodium content was reduced to nil.

Phosphorus, which is not a metal, is indicated in Table X since it does affect the weight of the ash. Since more than half of the weight of the ash in the oil after the second-stage treatment is represented by phosphorus, the actual metals content of the oil at this point is about 0.02 percent. The tremendous reductions in metals content of the oil, which parallel closely the reduction in ash content of the treated oil, clearly demonstrate the worth of

our process in recovering valuable metals, as well as in recovering valuable high viscosity index oils.

The presence of metals in a used lubricating oil makes the oil very difficult to treat by conventional refinery processes. By greatly reducing the metals content of a used lubricating oil in accord with the present process, the resulting oil may then be treated further using conventional refinery processing, such as distillation, hydro-treating, etc.

As illustrated by the foregoing discussion and the Examples, the present process provides a solution to the long-standing problem of recycling used lubricating oils. Thus, the use of the process will make a substantial contribution to environmental quality by providing a reduction in pollution of the air or water from the burning or disposal of used lubricating oils. Further, the present process represents a substantial contribution to the conservation of natural resources since it enables the reuse of relatively scarce high viscosity index oils which are needed for automotive lubrication.

We claim:

1. A method of purifying a used lubricating oil comprising:
  - admixing the used lubricating oil with a mutually soluble predominantly hydrocarbon liquid diluent;
  - admixing the diluted lubricating oil with a water-miscible alcohol and water mixture containing a small amount of an acid; and
  - centrifuging to remove sludge and metal compounds from the oil and to separate the diluted oil phase from the alcohol-water phase.
2. The method of Claim 1 wherein the predominantly hydrocarbon liquid diluent has a boiling range within the temperature region of about 100° F. to about 500° F.
3. The method of Claim 1 wherein the ratio of the predominantly hydrocarbon liquid diluent with respect to the used lubricating oil being treated ranges from about 2:1 to about 1:2 by volume.
4. The method of Claim 1 wherein the quantity of the acid is sufficient to displace polyvalent metal ions from the various metallic soaps contained in the used lubricating oil undergoing treatment.
5. The method of Claim 3 wherein the water-miscible alcohol is methanol, ethanol, isopropyl alcohol, *n*-propyl alcohol, *sec*-butyl alcohol or *tert*-butyl alcohol.
6. The method of Claim 3 wherein the water-miscible alcohol is isopropyl alcohol, ethanol, *tert*-butyl alcohol or *n*-propyl alcohol.
7. The method of Claim 6 wherein the water-miscible alcohol-water mixture contains from about 40 to about 60% by volume of the alcohol.
8. The method of Claim 3 wherein about one-half to about one volume of the water-miscible alcohol-water mixture are employed for each volume of the diluted lubricating oil.
9. The method of Claim 5 wherein about one-half to about one volume of the water-miscible alcohol-water mixture are employed for each volume of the diluted lubricating oil.
10. The method of Claim 6 wherein about one-half to about one volume of the water-miscible alcohol-water mixture are employed for each volume of the diluted lubricating oil.
11. The method of Claim 7 wherein about one-half to about one volume of the water-miscible alcohol-water mixture are employed for each volume of the diluted lubricating oil.
12. The method of Claim 1 wherein the acid is a mineral acid.
13. The method of Claim 12 wherein the acid is hydrochloric acid, nitric acid, phosphoric acid or sulfuric acid.
14. The method of Claim 6 wherein the acid is a mineral acid.

15. The method of Claim 14 wherein the acid is hydrochloric acid, nitric acid, phosphoric acid or sulfuric acid.

16. The method of Claim 1 including the steps of: distilling the diluted oil phase obtained from the centrifuging to obtain a light naphtha cut, and recycling the light naphtha cut to the process for use as the predominantly hydrocarbon liquid diluent.

17. A method of purifying a used lubricating oil comprising:

admixing the used lubricating oil with a mutually soluble predominantly hydrocarbon liquid diluent with the volume ratio of liquid diluent to used lubricating oil ranging from about 2:1 to about 1:2 and the liquid diluent having a boiling range within the temperature region of about 100° F. to about 500° F.; admixing the diluted lubricating oil with a mixture of isopropyl alcohol, ethanol, *n*-propyl alcohol, or *tert*-butyl alcohol and water which contains a small amount of an acid with about one-half to about one volume of the alcohol-water mixture being employed for each volume of the diluted lubricating oil, and centrifuging to remove sludge and metal compounds from the oil and to separate the diluted oil phase from the alcohol-water phase.

18. The method of Claim 17 wherein the acid is a mineral acid.

19. The method of Claim 18 wherein the acid is hydrochloric acid, nitric acid, phosphoric acid or sulfuric acid.

20. The method of Claim 17 wherein the quantity of the acid is sufficient to displace the polyvalent metal ions from the various metallic soaps contained in the used lubricating oil undergoing treatment.

21. The method of Claim 17 wherein the alcohol-water mixture contains from about 40 to about 60% by volume of alcohol.

22. The method of Claim 1 wherein said alcohol is a mixture of water miscible alcohols.

23. A multistage method of purifying a used lubricating oil comprising:

admixing the used lubricating oil with a neutrally soluble predominantly hydrocarbon liquid diluent; admixing the diluted lubricating oil with a water-miscible alcohol and water mixture containing a small amount of an ammonium or alkali metal base; centrifuging to remove sludge and metal compounds from the oil and to separate a first diluted oil phase from the alcohol-water phase;

5

10

15

20

25

30

35

40

45

50

admixing a water-miscible alcohol and water mixture containing a small amount of an acid with the first diluted oil phase or a mixture of a mutually soluble predominantly hydrocarbon liquid diluent with a purified lubricating oil from said first phase; and centrifuging to remove sludge and metal compounds from the oil and to separate a second diluted oil phase from the alcohol-water phase.

24. The method of Claim 23 wherein the predominantly hydrocarbon liquid diluent has a boiling range within the temperature region of about 100° F. to about 500° F.

25. The method of Claim 23 wherein the quantity of the ammonium or alkali metal base is sufficient to displace polyvalent metal ions from the various metallic soaps contained in the used lubricating oil undergoing treatment.

26. The method of Claim 23 wherein the water-miscible alcohol is methanol, ethanol, isopropyl alcohol, *n*-propyl alcohol, *sec*-butyl alcohol or *tert*-butyl alcohol, or mixtures thereof.

27. The method of Claim 23 wherein the base is sodium carbonate, potassium carbonate, or sodium phosphate.

28. The method of Claim 23 wherein the quantity of acid is sufficient to displace metallic ions from the first diluted oil phase or a mixture of a mutually soluble predominantly hydrocarbon liquid diluent with a purified lubricating oil from said first phase.

29. The method of Claim 23 wherein the acid is a mineral acid.

30. The method of Claim 29 wherein the acid is hydrochloric acid, nitric acid, phosphoric acid or sulfuric acid.

#### References Cited

##### UNITED STATES PATENTS

|           |         |                   |         |         |
|-----------|---------|-------------------|---------|---------|
| 2,376,418 | 5/1945  | Clark et al.      | -----   | 208—181 |
| 1,281,354 | 10/1918 | Handy             | -----   | 208—183 |
| 1,707,671 | 4/1929  | Aycock et al.     | -----   | 208—183 |
| 3,639,229 | 2/1972  | Brownawell et al. | 208—181 |         |
| 1,871,682 | 8/1932  | Ford et al.       | -----   | 208—180 |

##### FOREIGN PATENTS

|         |         |               |       |         |
|---------|---------|---------------|-------|---------|
| 742,909 | 11/1952 | Great Britain | ----- | 208—183 |
|---------|---------|---------------|-------|---------|

DELBERT E. GANTZ, Primary Examiner

J. M. NELSON, Assistant Examiner

U.S. CL. X.R.